

J. L. R. HAYDEN.  
ARC LIGHT ELECTRODE.  
APPLICATION FILED JULY 16, 1909.

1,082,950.

Patented Dec. 30, 1913.

FIG. 2



FIG. 1



WITNESSES:

J. Earl Ryan  
J. Ellis Elmer

INVENTOR:

JOSEPH L. R. HAYDEN,  
BY ALBERT S. DANI,  
ATTY.

# UNITED STATES PATENT OFFICE.

JOSEPH L. R. HAYDEN, OF SCHENECTADY, NEW YORK, ASSIGNOR TO GENERAL ELECTRIC COMPANY, A CORPORATION OF NEW YORK.

## ARC-LIGHT ELECTRODE.

1,082,950.

Specification of Letters Patent. Patented Dec. 30, 1913.

Application filed July 15, 1908. Serial No. 507,690.

To all whom it may concern:

Be it known that I, JOSEPH L. R. HAYDEN, a citizen of the United States, residing at Schenectady, in the county of Schenectady and State of New York, have invented certain new and useful Improvements in Arc-Light Electrodes, of which the following is a specification.

My invention has reference to improvements in arc light electrodes composed mainly of two or more metallic oxids and which electrodes are used particularly as cathodes in conjunction with an anode of carbon, of copper, or of other suitable metal.

The object of the invention is to secure greater uniformity of action of such electrodes than has heretofore been obtained, and this result I secure by making the electrode of a homogeneous mass of the ingredients used, by fusion, as will herein-after more fully appear.

The different metallic oxids of which such cathodes are composed have ordinarily different degrees of fusibility, and, owing to the incomplete mixture of the oxids obtained by the ordinary manner of mixing them, the different oxids fuse separately, that is to say, in succession, one after the other, in the pool which forms at the working end of the electrode; so that those compounds which fuse more readily are already in the fluid state when the more refractory ones are still solid. In consequence of this, the more refractory compounds do not furnish to the arc the amount of vapor or gas which is due to the proportion of these compounds in the composition of the electrode. Thus, for instance, in an electrode compounded of magnetite, rutile, chromite, and possibly some other slight admixture, like fluorid of potassium, it happens that when the magnetite is in a perfectly fluid state at the working end of the cathode the rutile is only imperfectly molten and the chromite may still be in a solid state. As a result of this the evolution of vapor from the rutile is retarded and the arc is either entirely or partially deprived during some stage of the operation of the luminosity which should be imparted to it by the titanium vapors.

The effect of the dissimultaneous fusion of the component parts of the compound is not observable at the beginning of the operation, but after the cathode has been used for some

time it manifests itself in the change of 55 color and dimming of the arc. Again, it may happen that the arc is maintained from the magnetite and rutile until these materials have been consumed at the point where the arc issues from the working end of the 60 electrode, and the arc must then feed upon the chromite particles until these in their turn are consumed. During this last phase of operation the arc assumes the dull bluish 65 tinge of the chromium arc. Its luminosity is diminished and it becomes hotter, and this higher temperature is deleterious to the positive electrode.

I have found that if the ingredients employed in the composition of the electrodes 70 are very uniformly mixed, the different constituents of the same, although of different degrees of fusibility, will in the arc practically fuse simultaneously, so that every constituent will give its proportional amount of 75 vapors to the arc.

In my application, Serial No. 448,797, filed August 17, 1908, I have described and claimed one mode of obtaining a uniform mixture of the component parts of an electrode compounded mainly of two or more metallic oxids, and my present invention is an improvement upon that set forth in said application.

My new process consists in fusing two or 85 more metal oxids, together with any other materials which are to enter into the composition of the electrode, into one homogeneous mass and casting electrode sticks from that fused mass. By this method of making electrodes the different metallic oxids form at the arcing end a pool which is composed of a fluid mixture of all the constituents, since now all of them fuse at substantially the same time, and the evolution of vapor or 90 gases from the same proceeds uniformly, each constituent giving vapors in proportion to its proportional quantity present in the mixture. No periodic dimming and change of color of light is observable in an electrode made in this manner.

An additional advantage of this invention is that it permits the use of a higher percentage of the more refractory metal oxids than has heretofore been practicable.

In the accompanying drawing, which forms a part of this specification, Figure 1 is an elevation of one form of my improved

electrode, and Fig. 2 is a longitudinal section of another form of electrode made in accordance with my invention.

In Fig. 1, the body 1 of the electrode is composed of a casting of a fused mixture of magnetite, rutile, chromite and some slight admixture, like fluorid of potassium, as a flux. The electrode is obtained by fusing these ingredients in the desired proportions to one homogeneous mass and then casting the electrode stick therefrom in any suitable mold. Owing to the comparative brittleness of this casting the electrode made in this manner will have to be comparatively short and thick, as indicated in the drawing; but much thinner and longer electrodes can be made by constructing them in the manner indicated in Fig. 2. The electrode shown in Fig. 2 is also made by casting in the manner hereinbefore described, except that the mold used becomes a part of the electrode, it being a metal tube, preferably an iron tube 2, which is closed at its lower end by an iron thimble 3, or in any other desired manner. In this case the fusion is purposely raised to a higher temperature than is absolutely necessary for casting, in order that the cast mass may become welded to the iron tube. This permits the making of long and thin electrodes, since the brit-

tleness of the cast material is neutralized in the whole stick by the soft metal shell.

While the invention is particularly useful in connection with electrodes containing two or more metal compounds that have different degrees of fusibility, it is also applicable and useful in connection with electrodes in which the materials employed fuse at substantially the same temperature. 35

Having now fully described my invention, 40 what I claim as new and desire to secure by Letters Patent of the United States, is:

1. The process of making arc light electrodes of two or more metallic compounds, which consists in fusing the ingredients to 45 one homogeneous mass and pouring the fluid mass at such temperature into a metal shell as to effect the welding of the mass with the shell.

2. An arc light electrode, formed of a 50 metal tube with a cast filling of a homogeneous mass containing two or more metallic compounds welded to the tube.

In witness whereof, I have hereunto set my hand this 12th day of July, 1909.

JOSEPH L. R. HAYDEN.

Witnesses:

HELEN ORFORD,  
THOMAS W. NOONAN.